

# United States Patent

## Odekerken

[15] 3,652,236

[45] Mar. 28, 1972

[54] **AN ARTICLE HAVING A LAYER CONTAINING NONCONDUCTIVE ORGANIC FIBERS AND METHOD OF PRODUCING**

[72] Inventor: **Jules Marie Odekerken**, Vught, Netherlands

[73] Assignee: **N. V. Research Holland**, Engelsweg, Hertogenbosch, Netherlands

[22] Filed: **Oct. 23, 1965**

[21] Appl. No.: **503,659**

[52] U.S. Cl. .... **29/195 P**, 204/41, 204/38 B,  
29/196.6, 29/194.2

[51] Int. Cl. .... **B32b 15/00**

[58] Field of Search .... **29/196.6, 194, 191.2; 204/40,  
204/41**

[56] **References Cited**

UNITED STATES PATENTS

3,152,971 10/1964 Tomaszewski ..... 204/41

|           |         |                  |          |
|-----------|---------|------------------|----------|
| 3,152,972 | 10/1964 | Brown .....      | 204/41   |
| 3,152,973 | 10/1964 | Tomaszewski..... | 204/41   |
| 3,268,423 | 8/1966  | Tomaszewski..... | 204/40   |
| 3,268,424 | 8/1966  | Brown .....      | 204/41   |
| 3,356,467 | 12/1967 | Brown .....      | 204/41   |
| 1,608,694 | 11/1926 | Cain .....       | 29/196.6 |
| 2,613,304 | 10/1952 | Colinet .....    | 29/195   |
| 2,792,624 | 5/1957  | Muller .....     | 29/191.2 |
| 3,291,578 | 12/1966 | Fahey .....      | 29/195   |

Primary Examiner—Hyland Bizot  
Attorney—Waters, Roditi, Schwartz & Nissen

[57]

### ABSTRACT

This invention pertains to a composite layered article and to a method for producing the article. The article consists of a body having an electrically conductive layer containing non-conductive organic fibers and a layer of chromium exterior to the fiber containing layer. There may be a metal layer intermediate the body and the organic fiber containing layer. The layers may be deposited electrolytically.

18 Claims, 2 Drawing Figures



PATENTED MAR 28 1972

3,652,236

FIG. 1



FIG. 2



AN ARTICLE HAVING A LAYER CONTAINING  
NONCONDUCTIVE ORGANIC FIBERS AND METHOD OF  
PRODUCING

This invention relates to the production of microporous chromium deposits and to articles having such deposits thereon.

It is already known from our British patent application 254/64 and our British publication, "Use of Co-Deposited Nonconducting materials to improve the Corrosion Resistance of Nickel-Chromium Electrodeposits," published in Electroplating and Metal Finishing, Volume 17 No. 1, Jan. 1964, pages 2-11, to produce microporous chromium deposits by applying onto an article, before the same is chromium-plated, metallic layers containing solid, nonconductive substances. As described on page 4 of the above publication, a disadvantage of this method is that the particle size of the nonconductive substances should be below about 10 microns, or the plating will have a rough surface.

It is an object of the invention to overcome the need for the use of solid nonconductive substances of small particle size in order to insure a smooth surface.

It is a further object of the invention to replace the known solid nonconductive substance with a class of substances which need not be of any specific prohibitive minimum size in order to confer a smooth surface finish to the protective layer.

Yet another object of the invention is to employ a class of substances as above-mentioned which are relatively inexpensive and readily available.

Still another object of the invention is to provide a relatively bright finish even when the content of the aforesaid class of substances is relatively high in order to produce an optimum microporous structure.

In accordance with the invention, it has been surprisingly found that the difficulty with regard to the small size required for the solid particles in order to insure smoothness of the plating can be overcome if the nonconductive materials which are used are organic fibers, as will be described hereinafter in greater detail.

Organic fibers may be subdivided into the following classes:

1. natural fibers
2. semi-synthetic fibers
3. synthetic fibers.

The class of natural fibers includes substances such as cotton (cellulose), wool (creatin), silk (chief ingredient fibroin, and albuminoid) kapok, flax, down, fur and the like.

The class of semi-synthetic fibers comprises fibers made synthetically from natural products, such as fibers produced from cellulose. Included in this class are also rubber fibers made from natural rubber.

The class of synthetic fibers includes fibers of polyamides polyesters, polyvinyl compounds, Latex, Kel F, silicones and the like.

The natural fibers usually having a thickness of 10-50 microns, the semi-synthetic fibers a thickness of 5-50 microns, and synthetic fibers are available with a thickness as small as 0.3 microns. The fibers with the above thicknesses are all effective for achieving their function as nonconductive materials, as will be shown more fully hereinafter. The length of the fibers can be determined by the user, since modern cutting devices afford accurate cutting of the fibers to a length of 5 microns. A very large number of organic fibers are commercially available in a sufficiently high grade; cellulose fiber, for example, is available in various lengths ranging from 40-110 microns under the name of Solka-Floc.

We have now discovered that these organic fibers, as described hereinbefore, in lengths ranging from 10 microns to as long as 300 microns, are an ideal expedient for producing microporous chromium deposits. The organic fibers may be directly used in a bright nickel bath, a semi-bright nickel bath or in a matte nickel bath. The chromium layer which is superposed will then be microporous and have a finish which is lustrous, semi-lustrous or matte. The open structure of the chromium plating can be determined by means of the Dubper-

nell test (Proc. American Electroplaters Soc. 1928, page 338).

When the content of organic fibers is increased to produce an optimum microporous structure, this will affect the luster if a bright nickel bath is used. There is first obtained a cloudy effect, and when the content of organic fibers is further increased, a uniform satin-like nickel deposit is obtained. Obviously, such a bath is unsuitable for producing a bright nickel deposit. It is, however, possible to first apply a bright nickel layer by means of a bright nickel bath which is free of fibers, and then apply a thin layer of a thickness, for example, of 0.1-3 microns, by means of a bright nickel bath having a high content of fibers, so that the luster of the basic bright nickel layer is not affected, whereafter finally the chromium layer is applied. This intermediate step between the application of the bright nickel layer and the chromium layer need not necessarily be effected with nickel. It is also possible to use any other metal, which, however, should preferably not be more oxidizable than nickel to prevent preferential corrosion of the metallic layer interposed between the chromium and the bright nickel. Also, this intermediate step need not be effected by means of electrolysis. The intermediate metallic layer may also be applied non-electrolytically. The organic fibers are kept in suspension by means of a stirrer or by air circulation or injection.

The invention is illustrated by the following examples, in which iron articles are subjected to the various treatments.

It should be understood, however, that the examples are merely illustrative and not intended to limit the invention in any way. It will be evident that the invention is not, for example, limited to iron as the base material, since the technical effect is obtained by virtue of the microporous chromium structure, which is separated from the base layer by means of a different layer, mostly nickel, so that a similar effect is obtained with other base materials, such as copper, brass, zinc, aluminum and even synthetic resin materials.

EXAMPLE I - BRIGHT NICKEL BATH INCORPORATING  
NATURAL FIBERS

In this example there was prepared a bath having the following composition and properties:

|                                                                                   |            |
|-----------------------------------------------------------------------------------|------------|
| Nickel sulphate                                                                   | 300 g./l.  |
| Nickel chloride                                                                   | 60 g./l.   |
| Boric acid                                                                        | 45 g./l.   |
| Butine diol                                                                       | 100 mg./l. |
| Saccharine                                                                        | 2 g./l.    |
| Sodium allyl sulfonate                                                            | 1 cc./l.   |
| Cellulose fiber BW 200, length<br>about 50 microns, thickness<br>about 17 microns | 50 g./l.   |
| pH                                                                                | 4          |
| Temperature                                                                       | 60° C.     |

x Cellulose fiber BW 200 is a product sold by Brown Co. of New York under the name Solka-Floc BW 200

In this bath an iron article is treated for 10 minutes at a current density of 5 a./dm.<sup>2</sup> until a bright nickel layer of 10 microns is obtained on the article, whereafter the article is plated with a chromium layer of 0.25 microns in a normal chromium bath. The article has a high brightness and a microporous chromium structure.

EXAMPLE II - SEMI-BRIGHT NICKEL BATH  
INCORPORATING NATURAL FIBERS

In this example there was prepared a bath having the following composition and properties:

|                               |            |
|-------------------------------|------------|
| Nickel sulphamate             | 300 g./l.  |
| Nickel chloride               | 10 g./l.   |
| Boric acid                    | 30 g./l.   |
| Formaldehyde                  | 50 mg./l.  |
| 2-butene-1,4-diol             | 20 mg./l.  |
| Chloral hydrate               | 100 mg./l. |
| Cellulose fiber, length about |            |

|                             |          |
|-----------------------------|----------|
| 50 microns, thickness about |          |
| 17 microns                  | 50 g./l. |
| pH                          | 4        |
| Temperature                 | 60° C.   |

In this bath an iron article is treated for 10 minutes at a current density of 5 a./dm.<sup>2</sup> until a nickel layer of 10 microns is obtained on the article, whereafter the article is plated with a chromium layer of 0.25 microns in a normal chromium bath. The article has a satin-like appearance and a microporous chromium structure.

#### EXAMPLE III - MATTE NICKEL BATH INCORPORATING NATURAL FIBERS

In this example there was prepared a bath having the following composition and properties:

|                               |           |
|-------------------------------|-----------|
| Nickel chloride               | 200 g./l. |
| Nickel sulphate               | 100 g./l. |
| Boric acid                    | 40 g./l.  |
| Cellulose fiber, length about |           |
| 50 microns, thickness         |           |
| about 17 microns              | 50 g./l.  |
| pH                            | 4.5       |
| Temperature                   | 50° C.    |

In this bath an iron article is treated for 10 minutes at a current density of 5 a./dm.<sup>2</sup> until a nickel layer of 10 microns is obtained on the article, whereafter the article is plated with a chromium layer of 0.25 microns in a normal chromium bath. The article has a matte finish and a microporous chromium structure.

#### EXAMPLE IV - BRIGHT NICKEL BATH INCORPORATING NATURAL FIBERS

Cellulose fiber BW200 in a concentration of about 100 g./l. in a bath of the following composition produces a cloudy effect; in a concentration of 150 g./l., however, a uniform satin-like finish is obtained.

|                               |            |
|-------------------------------|------------|
| Nickel sulphate               | 100 g./l.  |
| Nickel chloride               | 200 g./l.  |
| Boric acid                    | 45 g./l.   |
| Butine diol                   | 100 mg./l. |
| Succharine                    | 2 g./l.    |
| Sodium allyl sulpphonate      | 1 cc./l.   |
| Cellulose fiber, length about |            |
| 50 microns, thickness about   |            |
| 17 microns                    | 150 g./l.  |
| pH                            | 4          |
| Temperature                   | 60° C.     |

In this bath an iron article is treated for 5 minutes at a current density of 10 a./dm.<sup>2</sup> until a nickel layer of 10 microns is obtained on the article, whereafter the article is plated with a chromium layer of 0.25 microns in a normal chromium bath. The result is a satin-like or semi-bright finish and a 55 microporous chromium structure.

#### EXAMPLE V

An iron article is covered with a bright nickel layer of 9 microns in the bath of Example I without the cellulose, and then with 1 micron of the bath in Example IV. Finally, the article is covered with 0.25 micron of chromium. The article has a bright appearance and the chromium layer is microporous.

#### EXAMPLE VI

An iron article was coated with a layer of bright nickel of 9 microns by means of the bath of Example I, but without the cellulose, and then with 1 micron of nickel by means of the bath in Example IV containing, instead of cellulose fiber, wool fiber in a concentration of 100 g./l., the fibers having a thickness of about 20 microns and a length of about 120 microns. Thereafter, the article is covered with 0.25 micron of chromium. The result is a microporous chromium structure and a high brightness.

#### EXAMPLE VII

An iron article was covered with a bright nickel layer of 9 microns by means of the bath of Example I without the cellulose and then with 1 micron of nickel by means of the bath in Example IV, containing acetate cellulose fiber instead of cellulose. The fibers have a thickness of about 12 microns and a length of about 50 microns, and the concentration is 125 g./l. Thereafter the article is covered with 0.25 micron chromium. The result is a microporous chromium layer of high brightness.

#### EXAMPLE VIII

An iron article was covered with a layer of 9 microns of bright nickel by means of the bath of Example I without the cellulose fiber, and then is treated in the following electrolytic bath

|    |                                   |           |
|----|-----------------------------------|-----------|
| 20 | Cobalt chloride                   | 100 g./l. |
|    | Sodium Tungstate                  | 45 g./l.  |
|    | Rochelle salt                     | 400 g./l. |
|    | Ammonium chloride                 | 50 g./l.  |
| 25 | Nylon fiber thickness 0.5 microns |           |
|    | length 20 microns                 | 50 g./l.  |
|    | pH                                | 8.5       |
|    | Temperature                       | 90° C.    |

The article is treated for 1 minute at a current density of 1 a./dm.<sup>2</sup>. The article is then plated with 0.25 micron chromium. The result is a microporous chromium structure of high luster.

#### EXAMPLE IX

An iron article was covered with 9 microns bright nickel by means of the bath of Example I without the cellulose fiber, and then was treated in the following bath without the application of electric current for a period of 2 minutes.

|    |                                       |           |
|----|---------------------------------------|-----------|
| 40 | Nickel chloride                       | 30 g./l.  |
|    | Sodium citrate                        | 100 g./l. |
|    | Ammonium chloride                     | 50 g./l.  |
|    | Sodium hypophosphate                  | 20 g./l.  |
|    | PVC fiber, thickness 5 microns        | 100 g./l. |
|    | length 70 microns                     |           |
|    | Temperature                           | 90° C.    |
|    | pH (with NH <sub>4</sub> OH addition) | 9         |

45 The article is then covered with a chromium layer of 0.25 micron thickness. The result is a microporous chromium structure of high luster.

#### EXAMPLE X

50 For purposes of comparing the above articles produced by means of organic fibers with a microporous chromium layer, as described in the foregoing examples, several articles are coated with the following fiber-free bright nickel layers and finally also with 0.25 micron chromium layer.

- 10 microns bright nickel
- 20 microns bright nickel
- 40 microns bright nickel

All of the articles are then subjected to the corrodokote corrosion test (ASTM b 380/61/T).

The results are listed in the following table.

#### CORRODOKOTE TEST

| Article Produced by Example | % of rust after cycles |    |     |     |
|-----------------------------|------------------------|----|-----|-----|
|                             | I                      | II | III | IV  |
| I                           | 0                      | 0  | 0.1 | 0.3 |
| II                          | 0                      | 0  | 0   | 0.2 |
| III                         | 0                      | 0  | 0   | 0.2 |
| IV                          | 0                      | 0  | 0   | 0.1 |
| V                           | 0                      | 0  | 0   | 0   |
| VI                          | 0                      | 0  | 0   | 0.1 |
| VII                         | 0                      | 0  | 0   | 0.2 |
| VIII                        | 0                      | 0  | 0   | 0.2 |

|    |   |     |     |      |
|----|---|-----|-----|------|
| IX | 0 | 0   | 0   | 0.1  |
| Xa | 3 | 5   | 7   | 10   |
| Xb | 1 | 3   | 5   | 7    |
| Xc | 0 | 0.1 | 0.5 | ca 1 |

From the above it will be readily apparent that the surface deposits according to the invention are more corrosion resistant than the known deposits in which the organic fibers are absent. Moreover, this increase in corrosion resistance is present even when the nickel base layer of the known deposits is increased substantially in thickness.

Thus there can be obtained, according to the invention, a smooth chromium deposit of any desired luster which is highly corrosion resistant and microporous as a result of the incorporation of an organic fiber in a nickel layer beneath the chromium layer.

In Examples I-IV the brightness of the bath is a function of the quantity and type of brightness employed. Thus the high brightness of the article obtained according to Example I owes its existence to the presence of butine diol in the bath, while the satin-like appearance of the article obtained according to Example II is the result of the presence of 2-butene-1,4-diol. The bath described in Example III does not contain any brighteners so that the article obtained according to that Example has a mat finish.

The invention is next illustrated in conjunction with the attached drawing, wherein:

FIG. 1 is a cross-section view showing a first embodiment of microporous chromium deposit according to the invention; and

FIG. 2 is a second embodiment thereof.

In FIG. 1 there is shown an article 1, having an outer surface on which is applied a base layer 2. The base layer contains organic fibers 3 of the type as mentioned hereinbefore. Applied to the base layer 2 is a chromium layer 4 which is conferred with the microporous smooth surface. FIG. 1 represents the article with the deposit thereon, as shown in Examples I-IV.

In FIG. 2 there is illustrated the deposit as shown in Examples 5-9, wherein on the surface of the article 1' there is placed a base layer 5 constituted of nickel without organic fibers therein. An intermediate layer 2' is placed on the layer 5 and in layer 2' are contained the organic fibers 3'. Applied to the outer surface of intermediate layer 2' is chromium layer 4'.

The chromium layer 4 or 4' is not closed, but it is microporous. This microporosity is caused by the fibers which are disposed wholly or partially at the surface of the layer 2 or 2' respectively and serving in that way as insulators so that at that location no chromium is deposited. Thus, the deposit by electroplating of the chromium layer is interrupted where the organic fibers project from the surface of the base or intermediate layer, whereby the desired microporous structure is obtained for the chromium layer.

Numerous modifications and variations of the disclosed methods of the invention will become apparent to those skilled in the art without departing from the scope and spirit of the invention as defined in the attached claims.

What is claimed is:

1. A method of applying a smooth microporous chromium deposit on an article, said method comprising: applying to said article a metallic base layer containing organic fibers of non-conducting materials having a length of from 10 to 30 microns, and thereafter electrolytically applying a chromium layer on the base layer.

2. A method as claimed in claim 1, wherein said fibers are selected from the group consisting of natural fibers, semisynthetic fibers and synthetic fibers.

3. A method as claimed in claim 1, wherein said base layer is electrolytically deposited on the article in a bath, said organic fibers being present in the bath in an amount from 50 to 150

g./l.

4. A method as claimed in claim 3, wherein said bath is a nickel bath.

5. A method as claimed in claim 1, wherein said base layer has a thickness of 10 microns and the chromium layer has a thickness of about 0.25 micron.

6. A method as claimed in claim 1, wherein said organic fiber is present in the base layer in an amount to provide a surface finish for the article which may vary from bright to matte finish.

7. A method of applying a bright, smooth microporous chromium deposit on an article, said method comprising: applying to said article a bright metallic base layer, applying a thin second metallic layer containing organic fibers of non-conductive material onto said first layer, said fibers having a length of from 10 to 300 microns and thereafter electrolytically applying a chromium layer on the second layer.

8. A method as claimed in claim 7, wherein said second layer has a thickness between 0.1 and 3 microns.

9. A method as claimed in claim 8, wherein said base layer is a bright nickel layer and said second layer is a nickel layer with said fibers.

10. A method as claimed in claim 8, wherein said second layer is applied by electrolytically depositing the same on the base layer.

11. A method as claimed in claim 8, wherein said second layer is applied by immersing the article with the base layer thereon in a treatment bath containing the organic fibers suspended therein.

12. A method of forming a corrosion-resistant microporous deposit on an article, said method comprising applying on said article a corrosion-resistant metallic base layer having organic fibers of a length from 10 to 300 microns dispersed therein, and applying by electrolytic deposition a metallic corrosion-resistant layer on the first said layer with a thickness substantially less than that of said first layer, the second of said layers being rendered microporous by the organic fibers in the base layer.

13. An article having a deposit thereon, said deposit comprising an electrically conductive base layer on said article containing nonconductive organic fibers dispersed therein such that at least some of said fibers project through the surface of said base layer, and a layer of chromium on said base layer, the latter layer being interrupted at locations where the organic fibers project through the surface of the base layer.

14. An article as claimed in claim 13, wherein said base layer is a nickel layer having a thickness of 10 microns, the chromium layer having a thickness of 0.25 microns.

15. An article having a corrosion-resistant deposit thereon, said deposit comprising a metallic base layer containing a random orientation of nonconductive organic fibers, said fibers having a length of 10 to 300 microns, and an electrolytically deposited chromium layer on said base layer, said chromium layer being microporous by virtue of interruptions therein caused by the projection of at least some of the organic fibers from the surface of the base layer.

16. An article having a bright deposit thereon, said deposit comprising a bright metallic base layer, an intermediate layer on said base layer containing organic fibers dispersed therein, at least some of which project from the surface of the intermediate layer, and a microporous chromium layer on the intermediate layer.

17. An article as claimed in claim 16, wherein said intermediate layer is relatively thin compared to said base layer.

18. An article as claimed in claim 17, wherein said base layer is a nickel layer having a thickness of 9 microns and the intermediate layer is also nickel but of a thickness of 1 microns, the chromium layer having a thickness of 0.25 micron.